

Jan. 6, 1931.

F. C. OVERBURY

1,788,121

LAMINATED ROOFING

Filed March 2, 1926



Fig. 1



Fig. 2



Fig. 3



Fig. 4

Inventor:

Frederick C. Overbury,  
by  
Eight Brown Trunk Company  
Atty.

## UNITED STATES PATENT OFFICE

FREDERICK C. OVERTBURY, OF HILSDALE, NEW JERSEY, ASSIGNOR, BY MESNE ASSIGNMENTS, TO THE PATENT AND LICENSING CORPORATION, OF BOSTON, MASSACHUSETTS, A CORPORATION OF MASSACHUSETTS

## LAMINATED ROOFING

Application filed March 2, 1926. Serial No. 91,752.

This invention relates to prepared roofing and especially to comparatively thick and heavy roofing material of the laminated type, an object of the invention being to provide a laminated material which will not readily delaminate and which will have a structure tending to prevent curling. In general, thick roofing material presents distinct advantages over the relatively thin material which is widely used. It lies more securely against the lower courses, is less liable to be raised or bent by wind pressure, is less liable to be distorted by heat or moisture, and presents a better appearance. The chief difficulty which has been encountered in attempting to make thick roofing material by bringing together lamina of the usual weight of material is that roofing units so made have had a tendency to delaminate under the action of the weather. The present invention provides means to anchor the lamina firmly together to counteract the delaminating effects of the weather.

On the drawing,—

Fig. 1 is a diagrammatic representation of apparatus used in carrying out the invention;

Fig. 2 is a fragmentary showing of portions of two sheets of roofing base used in a preferred embodiment of the invention;

Fig. 3 shows a fragment of one form of the completed product; and

Fig. 4 shows a fragment of a slightly different form of the product.

Referring to the drawing in detail, 10 and 11 represent rolls of roofing base, such, for example, as the felt ordinarily used in preparing roofing, supported by a suitable standard 12. A saturating tank 13 is shown conventionally with rolls 14 to press out the surplus saturant from the sheet emerging from the container. The material in rolls 10 or 11 may be previously saturated or not, as desired. If not previously saturated, one or both of the sheets may be passed through the tank 13. As shown in the drawing, one sheet is saturated in the tank 13 while the other is led directly to the coating device, but with the addition of more guide and press rolls the upper sheet may readily be saturated in the tank 13. If either or both of the sheets are saturated after being drawn from their rolls 10, 11, suitable cooling

means, indicated at 25, is preferably provided before the coating compound is applied.

Before being coated, one or both of the sheets should be perforated. This may be done as by a perforator, conventionally indicated at 8, 9, after the sheet leaves rolls 10 or 11, but it is preferable to perforate one or both sheets at the paper mill so that the cut-out portions may be recovered at once in unsaturated condition, so that they can be put back immediately into the beater to prevent waste of material.

After the desired steps of perforating, saturating and cooling have been carried out on the sheets, they may be brought together by suitable guide rolls 15. A coating compound such as blown asphalt, or its equivalent, may then be applied to the outer surfaces of the sheets and also between the two. The latter coating may be supplied by a suitable spout 16 another spout 17 being provided to supply coating material for the upper surface of the upper sheet, and a roll 18 being positioned to dip into coating material 19 and apply the same to the under surface of the lower sheet. The sheets are together passed between the coating roll 18 and an upper roll 20, which remove surplus coating material and bring the sheets into more intimate contact. Comminuted material of any kind, such as crushed slate, may be supplied to one surface of the combined sheet from any suitable hopper, such as 21, the grit being rolled into the surface of the coating by press rolls 22. Grit may also be applied to the other surface of the combined sheet, if desired, and in any suitable way, after which the sheet may be cut into strips or individual shingles, or otherwise treated.

Figs. 3 and 4 show a fragmentary section of two preferred forms of laminated sheets which may be produced by the method recited. The form shown in Fig. 3 comprises one perforated sheet 30 and one unperforated sheet 31 of roofing base with the coating material 32 between the sheets and both sides thereof, the upper coating having a layer of grit 33 applied thereto. The form shown in Fig. 4 comprises two sheets 30 of roofing base, both of which are perforated. As will

be evident from Figs. 3 and 4, the coating material which is rolled over the surfaces of the laminations will be forced into the perforations so that the coatings on the different surfaces will be bonded by the element of coating material filling the perforations. This structure tends to prevent delamination.

Having thus described an embodiment of this invention, it should be evident to those skilled in the art that various changes and modifications may be made therein without departing from its spirit and scope as defined by the appended claims.

I claim:

15. 1. Laminated roofing material comprising a plurality of sheets of saturated roofing felt, layers of high melting-point asphalt between consecutive sheets of saturated felt and covering the outer faces thereof, at least one of said saturated sheets having perforations therethrough, elements of high melting-point asphalt extending through said perforations and bonding consecutive layers of asphalt on either side of the perforated and saturated sheet, and a layer of comminuted grit surfacing on one side of the laminated sheet.

20. 2. Laminated roofing material comprising a plurality of sheets of saturated roofing felt, each of said saturated sheets having perforations therethrough, layers of high melting-point asphalt between consecutive sheets and covering the outer faces thereof, elements of asphalt extending through said perforations and binding together all said layers of asphalt, and a layer of grit surfacing on one side of the laminated sheet.

In testimony whereof I have affixed my signature.

40 FREDERICK C. OVERBURY.

45

50

55

60

65